

J. R. Haskell.  
Paper Making.

N<sup>o</sup> 63,044

Patented Mar. 19, 1867.



Witnesses

W. W. Downing  
S. F. Elliott

Inventor;  
James R Haskell

# United States Patent Office.

JAMES R. HASKELL, OF NEW YORK, N. Y.

Letters Patent No. 63,044, dated March 19, 1867.

## IMPROVED MODE OF TREATING AND SEPARATING VEGETABLE FIBRES.

The Schedule referred to in these Letters Patent and making part of the same.

### TO ALL WHOM IT MAY CONCERN:

Be it known that I, JAMES R. HASKELL, of the city, county, and State of New York, have invented a new and improved Mode of Treating Vegetable Fibrous Substances; and I do hereby declare that the following is a full and exact description of the same.

The nature of my invention consists of a cheap and expeditious mode of reducing cane, crude hemp-stalks, and other fibrous substances to fibre, to be used in the arts.

To enable others skilled in the art to use my invention, I will proceed to describe the operation of my process, reference being had to the drawing hereto attached of an apparatus in which a portion of my process can be carried on; although I do not confine myself to this particular form, as it is obvious that the object sought can be accomplished in other ways besides that shown in the drawing.

The drawing represents a boiler, A, and reservoir, H, the boiler being connected through the pipe D with a steam boiler, not shown. The cane, crude hemp-stalks, or other fibrous material to be treated, may be flattened by being passed between rollers or not, according to the nature of the plant. First, I put the material in a vat or other suitable receptacle, and steep or boil it in lime-water for about four hours, more or less, for the purpose of softening the structure and neutralizing the acids contained in the sap of the plant, and extracting coloring matter. Second, I next pass the material between rollers for the purpose of squeezing out such mucilaginous substances as may have been eliminated by the action of the lime-water and heat. Third, I next put the material into the boiler A (see drawing) through the man-hole B, which is then tightly covered with the man-hole plate. Steam at a pressure of about two atmospheres is then let into the boiler A through the pipe and stop-cock D. The air and condensed water are next drawn off through the pipes I and E. F is the valve and opening through which the contents of the boiler A are discharged. After steaming the material for about one-half hour, more or less, for the purpose of opening and extending the pores or tubes of the plant and expelling the air from the same, the stop-cocks I, E, and D are closed, and an alkaline or caustic alkaline solution contained in the reservoir H is next turned on through the stop-cock and pipe C and rose-head  $\alpha$ , when a shower of cold lye is rained on the material in the boiler, which causes a rapid condensation of all the steam confined in the boiler and pores or tubes of the fibrous material under treatment, causing a vacuum or partial vacuum in the same, which is immediately filled with the alkaline solution. Steam is then let on again through the pipe and stop-cock D, and the material is boiled under a pressure of about two atmospheres for about two hours, more or less, for the purpose of further freeing the material from gum and coloring matter. Fourth, I next pass the material again between rollers, for the purpose of squeezing out the alkaline solution and spreading out and separating the fibres. The product can be used for paper making, textile or other purposes, in the usual manner. In the case of crude hemp-stalks, the product, as it comes from the rollers the last time, can be put into a beating engine or grinder, and the entire plant (including the long fibre on the outside and the short fibre of the woody portion or "shove") can be made into paper.

What I claim as my invention, and desire to secure by Letters Patent, is—

1. The mode of producing a vacuum or partial vacuum by first steaming the vegetable fibrous material under pressure and expelling the air, and then condensing the steam with a shower of cold lye, (which causes a rapid absorption of the lye in every part of the plant,) in the manner and for the purposes substantially as hereinbefore described.
2. I claim the mode of treating vegetable fibrous substances in the form and manner and for the purposes substantially as hereinbefore described.

JAMES R. HASKELL.

Witnesses:

W. W. DOWNING,  
S. B. ELLIOTT.